# EUROPEAN PATENT SPECIFICATION

(11) **EP 0 268 319 B1**
(45) Date of publication and mention of the grant of the patent: **06.05.1992**
(21) Application number: 87202092.0
(22) Date of filing: 30.10.1987
(51) Int. Cl.: C25B 1/00, C25C 1/10

(54) **Method for extracting Mn metal and manganese dioxide from divalent Mn salt solutions**
Verfahren zur Gewinnung von Mangan-Metall und Mangan-Dioxid aus zweiwertigen Mangansalzlösungen
Procédé d'extraction de manganèse et de dioxyde de manganèse à partir de solutions de sel de manganèse divalent

(30) Priority: 11.11.1986 IT 2228786
(43) Date of publication of application: 25.05.1988
(73) Proprietor: NUOVA SAMIM S.p.A., 20153 Milano (IT)
(72) Inventor: Guerriero, Renato, I-30170 Mestre Venice (IT); Vittadini, Italo, I-30170 Mestre Venice (IT)
(74) Representative: Roggero, Sergio

(56) References cited:
- US-A- 2 417 259
- US-A- 3 790 458
- CHEMICAL ABSTRACTS, vol. 108, no. 3, February 1988, page 568, abstract no. 64666c, Columbus, Ohio, US; & JP-A-85 104 334 (FUJIAN REACHER'S UNIVERSITY)
- CHEMICAL ABSTRACTS, vol. 79, no. 16, 22nd October 1973, page 548, abstract no. 99888m; & SU-A-380 742 (LENIN, V.I., GEORGIAN POLYTECHNIC INSTITUTE) 20-07-1970

## Description

This invention relates to a method for simultaneously extracting Mn metal and manganese dioxide in gamma form from divalent manganese salt solutions.

More particularly, the invention relates to a method for simultaneously extracting Mn metal and manganese dioxide in gamma form from manganese sulphate solutions.

The description given hereinafter refers to this second case, which is that of greatest interest.

The known art described separate methods for producing manganese dioxide or manganese metal.

Manganese dioxide is used in dry batteries in intimate mixture with graphite or acetylene black.

Preferably, manganese dioxide for batteries is in gamma form, and this can be obtained electrolytically by the following production process.

The overall electrochemical reaction on which manganese dioxide production is based is as follows:
- at the anode:: $\text{2Mn²⁺ → 2Mn³⁺ + 2e}$
$\text{2Mn⁺³ ⇄ Mn⁴⁺ + Mn⁺²}$
$\text{Mn⁺⁴ + 2H₂O → MnO₂ + 4H⁺}$
- at the cathode:: $\text{2H⁺ + 2e → H₂}$

The production process comprises the following steps:
1) Preparing the solution to be electrolysed
2) Electrolysis
3) Recovering the crude manganese dioxide
4) Treatment to obtain the commercial product

### Preparation of the solution:

The manganese salt which is dissolved in the electrolyte is the sulphate. It is obtained from various raw materials, those mostly used being the manganese minerals pyrolusite and rhodochrosite. A description of the preliminary heat treatments will be omitted for brevity. It will merely be stated that the crude manganese oxide is reacted with sulphuric acid, and the manganese sulphate solution formed is purified because minerals based on manganese dioxide generally have a certain heavy metals content. Purification with lime or limestone is followed by purification with calcium sulphide or hydrogen sulphide. The solution fed to electrolysis has an average MnSO₄ content of 80-150 g/l and an average H₂SO4 content of 50-100 g/l. A further component is ammonium sulphate (120-150 g/l) to act as a pH "stabiliser" during electrolysis.

### Electrolysis:

Electrolysis takes place in suitable cells under the following average conditions:
- current density at the anode: 70-120 A/m²
- voltage: 1.8-2.5 V
- electrolyte temperature: 90-95°C

To reduce the heat and evaporation losses, either closed cells are used or, more practically, the electrolyte is covered with a layer of oil or paraffin.

The electrolyte cycle can vary. In one cycle, the electrolyte is fed into the lower part of the cells in a quantity of 3% of the entire volume per minute; every one or two hours the electrolyte is cleaned by feeding 10-20% of it to treatment with MnCO₃ or MnO, and replacing this with fresh electrolyte. In another cycle, electrolyte is fed in such a quantity that the spent electrolyte leaves the cells containing 50 g/l of MnSO₄; this is mixed with an equal quantity of fresh electrolyte containing 150 g/l of MnSO₄ and the mixture is returned to the cycle.

### Recovery of manganese dioxide from the electrodes and its treatment:

When the dioxide deposited on the electrodes has reached the scheduled thickness, the anode assembly is removed from the cell in order to recover the product. This operation, which can be carried out either manually or automatically, is the most onerous of the process.

The MnO₂ fragments obtained from the anode deposits are washed with water and ground to less than 74 microns. The powder is again washed a number of times to eliminate any remaining acidity, and is again dried at low temperature, namely 80-85°C. All the various process steps are important in terms of production economy and the quality of the commercial product. The electrolysis operating conditions are also determining with regard to product quality and electricity consumption.

Both the labour requirement and the electrode life depend on the method used for recovering the dioxide from the electrodes.

### Electrolysis apparatus:

The cells are normally rectangular steel tanks clad with material which is resistant to both corrosion and temperature and is of very low conductivity, such as glass-fibre reinforced resins, rubber or acid-resistant cement or brick.

The electrodes can be flat or round bars or tubes.

The cathodes are generally of graphite, lead or stainless steel. Graphite anodes are mostly used, as they tolerate high current density without becoming passive, but their mechanical strength falls progressively due to corrosive attack.

Lead anodes normally containing 3-8% of antimony have the drawback that at high current density they are subject to chemical attack and contaminate the dioxide produced. They have the advantage that when they are no longer usable the lead can be recovered by smelting. Titanium anodes would perhaps be the ideal, but certainly very costly; they have excellent mechanical stability and a useful life of some years; they tend to become passive, but this drawback can be obviated by careful monitoring of the current density and the H₂SO₄ concentration in the electrolyte.

The useful anode:cathode surface area ratio is about 2:1. The distance between anodes and cathode is about 25-50 mm. A production cell can contain as many as 220 graphite anodes (flat bars of 1100 x 175 x 25 mm) arranged in 44 rows of 5 anodes each.

The manganese dioxide obtained by known methods has an average chemical composition of 62% Mn by weight, of which 92% is in the form of MnO₂, 1.6% is in the form of soluble Mn and the remainder is in the form of oxides other than MnO₂, together with traces of As, about 0.0004/% of copper by weight, traces of Ni and Co, 0.0001-0.05% of Pb by weight, about 0. 02% of Fe, about 1.2% of SO₄ by weight, and about 0.01% of SiO₂ by weight, the remainder to 100% being oxygen.

Having described the conventional system for producing electrolytic MnO₂, the known processes for producing Mn metal will now be described, as the process according to the present invention relates to the simultaneous electrolytic production of MnO₂ and Mn.

### Electrolytic production of manganese

The solution to be electrolysed generally consist of manganous sulphate and ammonium sulphate, and is practically neutral. Cathodic electrodeposition in accordance with the overall reaction;

$\text{Mn²⁺ + H₂O → Mn + 2H⁺ + ½O₂}$

takes place under the following conditions.

| Conditions: | | |
|---|---|---|
| Catholyte: | Mn as MnSO₄ | 30-40 g/l |
| | (NH₄)₂SO₄ | 125-150 g/l |
| | SO₂ | 0.3-0.5 g/l |
| | pH | 6-7.2 |
| Anolyte: | Mn as MnSO₄ | 10-20 g/l |
| | H₂SO₄ | 25-40 g/l |
| | (NH₄)₂SO₄ | 125-150 g/l |
| Current density: | | 430-650 A/m² |
| Anode composition: | | Pb + 1% Ag |
| Cathode composition: | | Hastelloy or AISI 316 or Titanium |
| Cell voltage: | | 5.2 V |
| Diaphragm: | | acrylic, cotton |
| Current yield: | | 65-75% |

The following table shows the impurities usually contained.

| ELEMENT | CONTENT |
|---|---|
| Fe | 15 mg/l |
| Cu | 10 g/l |
| As | 5 g/l |
| Co | 25 g/l |
| Ni | 25 g/l |
| Pb | 25 g/l |
| Mo | 10 g/l |

A method has been surprisingly found, and constitutes the subject of the present invention, for simultaneously obtaining Mn metal and manganese dioxide, ie for combining the separate processes heretofore described, by electrolysing a manganese sulphate solution in an electrolytic cell provided with an anionic membrane.

The present invention provides a method for simultaneously obtaining Mn metal and manganese dioxide in gamma form according to present cl.1
The reaction which takes place at the anode is as follows:

$\text{2Mn²⁺ → 2 Mn³⁺ + 2e}$

The reaction which takes place at the cathode is as follows:

$\text{Mn²⁺ + 2e → Mn}$

The following hydrolysis reaction also takes place:

$\text{2Mn³⁺ + 2H₂O → MnO₂ + Mn²⁺ + 4H⁺}$

The electrolysis proceeds with the passage of SO₄²⁻ ions from the cathode compartment to the anode compartment of the cell divided by the anionic membrane.

The overall reaction which takes place during the electrolysis can be represented by the following equation:

$\text{2Mn²⁺ + 2H₂O → MnO₂ + Mn + 4H⁺}$

In a preferred embodiment of the method according to the present invention, the electrolysis is implemented with a cell which is shown diagrammatically on the accompanying figure.

The cell consists of a cylindrical container 1, particularly of PVC, in which a lead alloy anode 2 and a stainless steel cathode 3 are disposed.

The anode region 4 is separated from the cathode region 5 by an anionic membrane 6 having a funnel-shaped base.

The membrane 6 is of the aforesaid type, its purpose being to allow the SO₄²⁻ ions to pass from the cathode region to the anode region.

The feed to the anode region is represented by the reference numeral 7; the feed to the cathode region is represented by the reference numeral 8. The discharge from the cathode region is indicated by the reference numeral 9 and the discharge from the anode region is indicated by the reference numeral 10. The reference numeral 11 indicates the anode recycling, and 12 the feed and discharge pipes for the cooling water of the anode 2.

It should be noted that the height of the anode discharge offtake is adjustable so as to obtain a level difference between the free surface of the anolyte and that of the catholyte.

The conditions additional to the aforesaid under which the method according to the present invention is operated are as follows:
- anode current density between 3000 A/m² and 5500 A/m²
- cathode current density between 250 A/m² and 400 A/m²
- anolyte consisting of a solution containing 20-40 g/l of Mn and 100-300 g/l of H₂SO₄
- catholyte consisting of a solution containing 30-50 g/l of manganese and 150-200 g/l of ammonium sulphate, at a pH of between 6 and 7
- anolyte temperature between 15 and 30°C
- catholyte temperature between 20 and 35°C

Some examples are given hereinafter in order to better illustrate the invention, which however is not limited by them or to them. The described apparatus shown on the figure and comprising an anionic membrane is used in the examples.

| EXAMPLE 1 | | |
|---|---|---|
| Overall feed solution | Mn | 40 g/l |
| | (NH₄)₂SO₄ | 170 g/l |
| | SO₂ | 0.1 g/l |
| | pH | 6.3 |
| Cathode current density | | 350 A/m² |
| Temperature of cathode region | | 30°C |
| Anode current density | | 4500 A/m² |
| Temperature of anode region | | 30°C |
| Cathode current yield (Mn) | | 56% |
| Anode current yield (MnO₂) | | 83% |

| EXAMPLE 2 | | |
|---|---|---|
| Overall feed solution | Mn | 38 g/l |
| | (NH₄)₂SO₄ | 200 g/l |
| | SO₂ | 0.2g/l |
| | pH | 6.5 |
| Cathode current density | | 300 A/m² |
| Temperature of cathode region | | 28°C |
| Anode current density | | 3850 A/m² |
| Temperature of anode region | | 30°C |
| Cathode current yield (Mn) | | 60% |
| Anode current yield (MnO₂) | | 95% |

| EXAMPLE 3 | | |
|---|---|---|
| Overall feed solution | Mn | 42 g/l |
| | (NH₄)₂SO₄ | 150 g/l |
| | SO₂ | 0.1g/l |
| | pH | 6.1 |
| Cathode current density | | 400 A/m² |
| Temperature of cathode region | | 35°C |
| Anode current density | | 5100 A/m² |
| Temperature of anode region | | 30°C |
| Cathode current yield (Mn) | | 55% |
| Anode current yield (MnO₂) | | 93% |

| EXAMPLE 4 | | |
|---|---|---|
| Overall feed solution | Mn | 35 g/l |
| | (NH₄)₂SO₄ | 180 g/l |
| | SO₂ | 0.2g/l |
| | pH | 6.8 |
| Cathode current density | | 250 A/m² |
| Temperature of cathode region | | 22°C |
| Anode current density | | 3100 A/m² |
| Temperature of anode region | | 25°C |
| Cathode current yield (Mn) | | 58% |
| Anode currant yield (MnO₂) | | 89% |

## Claims

1. A process for electrolytically preparing metallic manganese and gamma manganese dioxide simultaneously by electrolyzing two streams of an aqueous solution of manganese salt separated by a porous membrane, characterized in that said separatory membrane consists of a hydrocarbon or a fluorocarbon polymer containing quaternary ammonium groups, the anolyte being an aqueous solution of manganese sulphate acidified by sulphuric acid and the catholyte being an aqueous solution of manganese sulphate acidified by sulphuric acid and supplemented by ammonium sulphate and SO₂, under an anodic current density of from 3000 A/m² to 5500 A/m² and a cathodic current density of from 250 A/m² to 400 A/m².

2. Process according to Claim 1, wherein the anolyte contains from 20 g/l to 40 g/l of Mn and from 100 g/l to 300 g/l of H₂SO₄.

3. Process according to Claim 1, wherein the catholyte contains from 30 g/l to 50 g/l of Mn and from 150 g/l to 200 g/l of ammonium sulphate, and has a pH of from 6 to 7.

4. Process according to Claim 1, wherein the anolyte temperature is of from 15°C to 30°C.

5. Process according to Claim 1, wherein the catholyte temperature is of from 20°C to 35°C.

## Patentansprüche

1. Verfahren zur gleichzeitigen elektrolytischen Herstellung von metallischem Mangan und gamma-Mangandioxid durch Elektrolyse zweier Ströme einer wäßrigen Lösung eines Mangansalzes, die durch eine poröse Membran getrennt sind, durch gekennzeichnet, daß diese Separatormembran aus einem Kohlenwasserstoff- oder einem Fluorkohlenstoffpolymer mit einem Gehalt an quaternären Ammoniumgruppen besteht, wobei der Anolyt eine wäßrige Lösung von mit Schwefelsäure angesäuertem Mangansulfat ist und der Katholyt eine wäßrige Lösung von Mangansulfat ist, das mit Schwefelsäure angesäuert und mit Ammoniumsulfat und SO₂ ergänzt ist, bei einer Anodenstromdichte von 3.000 A/m² bis 5.500 A/m² und einer Kathodenstromdichte von 250 A/m² bis 400 A/m².

2. Verfahren nach Anspruch 1, worin der Anolyt 20 g/l bis 40 g/l Mn und 100 g/l bis 300 g/l H₂SO₄ enthält.

3. Verfahren nach Anspruch 1, worin der Katholyt 30 g/l bis 50 g/l Mn und 150 g/l bis 200 g/l Ammoniumsulfat enthält und einen pH-Wert von 6 bis 7 aufweist.

4. Verfahren nach Anspruch 1, worin die Anolyttemperatur 15°C bis 30°C beträgt.

5. Verfahren nach Anspruch 1, worin die Katholyttemperatur 20°C bis 35°C beträgt.

## Revendications

1. Procédé de préparation électrolytique simultanée de manganèse métal et de dioxyde de manganèse gamma, par électrolyse de deux courants d'une solution aqueuse de sel de manganèse, séparés par une membrane poreuse, caractérisé en ce que ladite membrane de séparation est constituée d'un polymère hydrocarboné ou fluorocarboné renfermant des groupes ammonium quaternaire, l'anolyte étant une solution aqueuse de sulfate de manganèse, acidifiée par de l'acide sulfurique, et le catholyte étant une solution aqueuse de sulfate de manganèse, acidifiée par de l'acide sulfurique, à laquelle on a ajouté du sulfate d'ammonium et du SO₂, la densité de courant anodique étant de 3000 A/m² à 5500 A/m² et la densité de courant cathodique étant de 250 A/m² à 400 A/m².

2. Procédé selon la revendication 1, dans lequel l'anolyte contient de 20 g/l à 40 g/l de Mn et de 100 g/l à 300 g/l de H₂SO₄.

3. Procédé selon la revendication 1, dans lequel le catholyte contient de 30 g/l a 50 g/l de Mn et de 150 g/l à 200 g/l de sulfate d'ammonium, et a un pH de 6 à 7.

4. Procédé selon la revendication 1, dans lequel la température de l'anolyte est de 15°C à 30°C.

5. Procédé selon la revendication 1, dans lequel la température du catholyte est de 20°C à 35°C.
